

March 9, 1926.

1,576,317

C. E. EKLIND

METHOD OF FORMING REINFORCED CASTINGS

Filed April 16, 1925



Fig. 2.



Fig. 5.



Fig. 6.



Fig. 7.



Fig. 3.



Fig. 4.



Inventor.  
Carl E. Eklind  
By Paul O. Pipel  
Atty.

## UNITED STATES PATENT OFFICE.

CARL E. EKLIND, OF BURWYN, ILLINOIS.

## METHOD OF FORMING REINFORCED CASTINGS.

Application filed April 16, 1925. Serial No. 23,469.

*To all whom it may concern:*

Be it known that I, CARL E. EKLIND, a citizen of the United States, residing at Berwyn, in the county of Cook and State of Illinois, have invented certain new and useful Improvements in Methods of Forming Reinforced Castings, of which the following is a full, clear, and exact specification.

My invention relates generally to a method and means for making reinforced castings and particularly to a method of forming such reinforced castings during the molding operation or manufacture thereof.

An object of this invention is to devise a simple and inexpensive method for reinforcing castings in the process of manufacture, and particularly strengthening such parts of castings as are subjected in service to the greatest stresses, to the end that objectionable strains and breakages in the castings during service are effectually prevented.

A further object is to form castings having strengthened portions formed during manufacture by means of inserts or inlays of tougher and greater stress and strain resisting quality than the main body of the casting.

Still another object of this invention is to have such strengthening inserts and inlays become an integral part of the casting which cannot become loose therefrom.

As the description hereof progresses, other objects and advantages should become obvious to anyone skilled in this art. While it should be understood that this invention is applicable to the manufacture of all kinds of castings, and especially metallic castings, nevertheless, I have chosen in the present preferred embodiment to illustrate the same in connection with the manufacture of improved castings for railway appliances, as this field presents a great variety of metallic, and particularly castings of ferrous metals, where the present improvement could be effectively employed.

Briefly stated, the invention comprises the following method of forming reinforced castings, wherein the mold is first prepared in the conventional manner. Reinforcing inserts or inlays of material tougher than the main body of the casting are then supported in proper position in the mold, the same having been preheated to a welding temperature, either heated before or after being placed in the mold in any suitable

manner, as by means of electricity, to such a temperature as will approximate as nearly as possible, without melting, the temperature of the metal to be poured into the mold. The metal to be poured is heated to a temperature in excess of its melting point and is then poured into the mold and around or against the insert or inlay which absorbs the excess heat of the poured metal, the two metals then welding together and adhering in a manner to form an integral, unitary casting.

As already stated this method could be advantageously employed in the railway car rigging art where such castings as car wheels, brake shoes, side truck frames and bolsters are subjected to great stresses causing many breakages, and accordingly I have chosen to illustrate in the accompanying drawings a car wheel and brake shoe to show the manner of strengthening such particular castings.

In the drawings,—

Fig. 1 is a sectional view of a conventional mold showing the manner of forming a reinforced car wheel therein;

Fig. 2 is a plan view illustrating a segmental fragment of one face of such wheel with the reinforcing inlay welded thereon;

Fig. 3 is a detail sectional view showing the inlay welded over the usual ribs or brackets of standard car wheels, and is taken along line 3—3 of Fig. 2, looking in the direction of the arrows;

Fig. 4 is a sectional detail of a wheel formed with reinforcing inserts rather than inlays and is a modification of the first disclosure;

Fig. 5 is a side view of a form of brake shoe with a reinforcing back piece cast integrally with its body;

Fig. 6 is a sectional view thereof along line 6—6 of Fig. 5, looking in the direction of the arrows; and

Fig. 7 is a similar view along the line 7—7 of Fig. 5, looking in the direction of the arrows.

To illustrate the improved method of casting better castings, a conventional two-part molding flash 10 is shown, the same being filled with sand and hollowed out in the usual way for pouring metal thereinto, such as cast iron, to mold the standard railway car wheel 11 shown therein. Each side edge 110 adjacent the flange of these standard cast iron wheels soon chips and fritters off due

to the strain of usage, and the object here is to strengthen these portions of the wheel in a manner to overcome this difficulty. Accordingly, there is placed in the mold, as shown, a pair of annular ring members 12 of tougher material than the wheel proper, such for example as wrought iron or open hearth steel, are placed in the mold as shown, the lower annulus lying properly in the mold hollow while the upper one must be supported by chaplets 13 of any suitable kind. Obviously, of course, these ring members must be shaped to conform with the faces of the marginal edges of the wheel adjacent the flange. These ring members then are connected in electric circuits, where they become in effect resistance elements, and by means of electric current of the necessary voltage are heated to a temperature as nearly as possible approximating the temperature of the molten metal to be poured to form the main body of the casting without melting and destroying the form of these rings. The circuit leads for the upper ring are shown at 14 while those for the lower ring are shown at 15. Both rings could, of course, be included in a single circuit, if desired. Insulated conductors 16 are employed to pass the current through the sand to the rings. When the rings are properly preheated the current may be cut off and the cast iron poured into the mold at 17 in the usual way, the metal completely filling the hollow in the mold and contacting the preheated rings of different material. The two metals are then permitted to cool slowly together to insure equal shrinkage, the metals in effect at their contacting surfaces securely welding or amalgamating together to form an integral wheel, which will be materially strengthened in those places where the stresses will be greatest. One face of the standard wheel is provided with the usual brackets or ribs 18, as shown, and the strengthening ring of different material, as shown in Figs. 1, 2 and 3, may be formed over these ribs. The chaplets 13 will become a part of the finished casting very likely, as they may be made to unite with either the ring or casting proper. The upper insulators 16 may be arranged to support these chaplets as shown. These strengthening inlays or rings may, of course, be preheated in any other way and may even be heated before being placed in the mold. Each insert or inlay ring could be of a different metal to meet any particular kind of stress; that is, the completed casting could be an integral unit of three different metals.

In Fig. 1, a chill 21 is shown in the mold for the purpose of chilling and hardening the wheel tread or tire, as is usually done. This will in no way interfere with the method herein disclosed.

Fig. 4 shows a modified wheel wherein the molten metal is cast completely around strengthening inserts by the present method. Here the inserts could be perforated so that the poured metal could take a better grip on the insert.

A brake shoe 19, as shown in Figs. 5, 6 and 7, having a main body of iron may also have a strengthening back 20 of tougher material, such as steel, integrally formed thereon by my method.

Obviously the method is applicable to the formation of any castings to be made of different metals and particularly in the integral formation of a tougher wearing or strain and stress resisting surface or part for such castings.

Striated surfaces and interlocking projections could also be formed on the surfaces of the reenforcing part to insure a tight weld with the main body of the casting, if desired.

The terms "weld" and "welding" herein employed are intended to mean the uniting of the different metals as by the adherence of one with the other due to the heat at their contacting surfaces and not in the sense of alloying the different metals. In practice the metal to be poured will be heated somewhat above its melting point so that its surplus heat will be absorbed by the reenforcing pieces to insure a better adherence between the different metals. This, for the reason that the inlay pieces 12 can be preheated only to a certain extent. They must not be heated too much lest they lose their shapes and they must, of course, also retain their positions in the mold, which they cannot do if heated too much. The superheat of the poured metal is absorbed by the inlays and they cannot then lose their preformed shapes because the poured metal fills the mold and holds them in position. With the inlays disposed on the outside as shown in Figs. 1, 2 and 3, the wheel is formed with a hard, tough, outer reenforced surface in a manner best conducive to resist wear and strain. Obviously, the inlays could be in the form of disks and form a cover for the entire face of the wheel.

Although I have illustrated the preferred embodiment of my invention, it will be evident that various changes in the method may be made without departing from the spirit of the invention, and, therefore, I do not limit myself to the exact disclosure made as indicated in the subjoined claims.

What I claim is:

1. The method of forming reenforced cast wheels comprising preheating preformed reenforcing pieces of one metal in a mold to substantially the highest temperature they will stand without losing their shapes, the pieces being so placed in the mold that one will be on the outside of each face of the

finished wheel, then pouring a molten metal of a different quality and at a temperature in excess of its melting point into the mold against and between the reenforcing pieces, 5 such reenforcing pieces absorbing such excess heat and welding with the poured metal, the metals then cooling and shrinking together to form an integral cast wheel having faces provided with exposed reenforcing 10 pieces.

2. The method of forming a reenforced cast wheel which consists in supporting preformed annular tough, ferrous pieces in a mold hollow, preheating the pieces in the 15 mold to the highest temperature which they will stand without losing their preformed annular shapes, then pouring a molten ferrous metal of a different quality at a temperature in excess of its melting point into 20 the mold hollow against the preformed pieces the pieces absorbing the excess heat of the poured metal and welding therewith,

the metals then cooling and shrinking together to form an integral cast ferrous wheel having exposed reenforcements thereon. 25

3. The method of forming reenforced castings having exposed reenforcing pieces, comprising properly supporting and positioning hard preformed reenforcing pieces of one metal in a mold hollow and preheating them 30 to a temperature which will transform them to a soggy state without destroying their shapes, then pouring a molten metal of a different quality and at a temperature in excess of its melting point into the mold 35 against the reenforcing pieces, the said pieces absorbing such excess heat and welding with the poured metal, the metals then cooling and shrinking together to form an integral casting having exposed 40 reinforcements thereon.

In testimony whereof I affix my signature.

CARL E. EKLIND.